

# UNITED STATES PATENT OFFICE.

HERRMANN WOLFF, OF NEW YORK, N. Y., ASSIGNOR OF TWO-THIRDS TO  
ALEXANDER MENKE AND HERMAN OPPENHEIMER, OF SAME PLACE.

## ARTIFICIAL FUEL.

SPECIFICATION forming part of Letters Patent No. 623,504, dated April 18, 1899.

Application filed April 20, 1898. Serial No. 678,250. (No specimens.)

*To all whom it may concern:*

Be it known that I, HERRMANN WOLFF, a citizen of Germany, and a resident of New York, county and State of New York, have 5 invented certain new and useful Improvements in Artificial Fuel, of which the following is a full, clear, and exact specification.

My invention relates to compounding of fuel materials; and it consists of a composition of matter suitable for use as fuel for any 10 and all such purposes as natural coal is used.

The composition consists of the following ingredients: coal-dust or pulverized lignite, pitch, wax-tailings, barium sulfate, and benzin, compounded as hereinafter described and 15 then formed into briquets of suitable size and shape and compressed in hydraulic press to render the composition absolutely compact and hard.

20 My newly-invented artificial fuel is capable of being stored or transported in the same manner as natural coal, will not disintegrate or decompose when exposed to air, heat, or moisture, and its capacity for producing heat 25 will not be affected by long storage. In this respect my compounded fuel is preferable to natural coal. Its heat-producing capacity is as great as that of best coal, and as it does not deteriorate it can be kept stored for an 30 indefinite period of time and under any conditions.

Another and also very important advantage of my compounded fuel is that when prepared as hereinafter described the briquets may be piled up in rows like building-bricks and kept for an indefinite time in 35 closed bunkers or bins without any danger of instantaneous combustion, nor will the fuel produce any explosive, combustible, or otherwise dangerous gases whatsoever.

The composition is compounded of the above-enumerated ingredients as follows: The coal-dust, eighty-nine parts, in weight, is mixed with six parts of finely-pulverized 40 pitch, and while the mixing is done the ingredients are heated to 100° Fahrenheit. At the same time wax-tailings, three parts, is melted by heating it slowly to boiling heat, approximately to 220° Fahrenheit, and then 45 one part of barium sulfate added thereto. When these two ingredients are thoroughly

55 united, the same are allowed to cool off to about 100° Fahrenheit. Then one part of benzin is added thereto and the fluid slowly reheated. Then the comixture of coal-dust and pitch is successively added thereto and the whole, while constantly kept warm, thoroughly mixed. The composition is then in a nearly plastic state and in condition to be formed into bricks or briquets by suitable machinery. The briquets, while yet warm, in forms are conveyed to a hydraulic press and there subjected to a pressure of approximately two thousand five hundred pounds per square inch, and after being thus compressed 60 are allowed to harden in the atmospheric air. The compounded fuel when dried is hard and compact, though not brittle, and may then immediately be used or stored.

With regard to the wax-tailings I desire to 70 state that though this ingredient is in itself meltable by heat it enters with the barium sulfate in some such chemical combination by which its capacity of being melted by heat is destroyed, and consequently when the fuel 75 is used in furnace its binding material does not melt and the briquets behave in fire the same as natural coal of very good quality. They do not disintegrate or bake. They burn 80 in the same manner as natural coal, slowly or fiercely, according to the quantity of the draft of air supplied to the furnace.

When using the term "coal" or "coal-dust" in this specification, it is to be understood as embracing not only anthracite or bituminous 85 or so-called "soft coal," but also lignite, which some experts believe to be a different substance from coal, whereas others hold it to be merely an imperfect kind of coal.

The relative quantity of the ingredients 90 may be varied; but the proportion as stated above will produce the best composition suitable as artificial fuel for any purpose for which natural coal can be used.

I claim as my invention, and desire to set 95 out by Letters Patent—

1. A composition of matter suitable for use as fuel, comprising coal-dust, pitch, wax-tailings, barium sulfate, and benzin.

2. A composition of matter suitable for use 100 as fuel, comprising eighty-nine parts of coal-dust, six parts of pitch, three parts of wax-

tailings, one part of barium sulfate and one part of benzin.

3. The process of producing artificial fuel, consisting first, of mixing dry coal-dust and finely-pulverized pitch in appropriate quantities and heating these ingredients to 100° Fahrenheit, second, melting a suitable quantity of wax-tailings by heating the same to 220° to 230° Fahrenheit and adding thereto, 10 while the heating is continued, barium sulfate; third, allowing the fluid to cool off to about 100° Fahrenheit, adding thereto benzin and then slowly reheating and mixing there-

with the coal-dust and pitch thoroughly, and fourth, forming and compressing the mixed 15 ingredients into briquets of suitable shape and size.

In witness that I claim the improvements described in the foregoing specification I have signed my name in the presence of two sub- 20 scribing witnesses.

HERRMANN WOLFF.

Witnesses:

HENRY SCHREITER,  
ROBERT VALENTINE MATHEWS.